

## UNITED STATES PATENT OFFICE

2,116,273

## ALUMINIUM ALLOY

Yonosuke Matuenaga, Naka-ku, Yokohama,  
Japan

No Drawing. Application November 12, 1936, Serial No. 110,552. In Japan May 13, 1935

1 Claim. (Cl. 75—141)

This application is a continuation-in-part of applicant's copending application Serial No. 78,721 filed May 8, 1936.

This invention relates to an aluminium alloy comprising main and auxiliary elements, the main element consisting of 2 to 5% magnesium, 6 to 14% zinc, 0.3 to 2% copper, 0.01 to 0.5% iron, 0.1 to 1.0% silicon and the rest substantially aluminium keeping the condition that the content of silicon is always greater than that of iron, while the auxiliary element consisting of a metal selected from the group of 0.1 to 1.0% manganese, 0.1 to 5% cobalt, 0.1 to 5% molybdenum, and 0.1 to 1.5% lithium. The new alloy may also contain a small quantity of vanadium, beryllium and tungsten in place of a part of aluminium. The object of the invention is to obtain a new aluminium alloy which has both a great tensile strength and a great elongation especially when subjected under heat treatment.

Examples of the alloy showing percentages of the elements employed and also tensile strength and elongation when the alloys are subjected under a mode of tempering and annealing are given as follows:

## Example 1

|                                       |      |      |
|---------------------------------------|------|------|
| Mg                                    | 2.5  | 2.5  |
| Zn                                    | 9.0  | 9.0  |
| Cu                                    | 0.5  | 1.0  |
| Fe                                    | 0.2  | 0.2  |
| Si                                    | 0.6  | 0.6  |
| Mn                                    | 0.8  | 0.8  |
| Al                                    | Rest | Rest |
| Tensile strength kg./cm. <sup>2</sup> | 60   | 63   |
| Elongation %                          | 15   | 17   |

## Example 2

|                                       |      |      |
|---------------------------------------|------|------|
| Mg                                    | 3.0  | 3.0  |
| Zn                                    | 7.0  | 7.0  |
| Cu                                    | 1.2  | 1.2  |
| Fe                                    | 0.3  | 0.3  |
| Si                                    | 0.8  | 0.8  |
| Co                                    | 1.0  | 2    |
| Al                                    | Rest | Rest |
| Tensile strength kg./cm. <sup>2</sup> | 57   | 59   |
| Elongation %                          | 11   | 9    |

## Example 3

|                                       |      |     |
|---------------------------------------|------|-----|
| Mg                                    | 3.0  | 3.0 |
| Zn                                    | 8.0  | 8.0 |
| Cu                                    | 1.0  | —   |
| Fe                                    | 0.2  | —   |
| Si                                    | 0.5  | —   |
| Mo                                    | 3.0  | —   |
| Al                                    | Rest | —   |
| Tensile strength kg./cm. <sup>2</sup> | 56   | —   |
| Elongation %                          | 10   | —   |

## Example 4

|                                       |      |     |
|---------------------------------------|------|-----|
| Mg                                    | 2.5  | 2.5 |
| Zn                                    | 9.0  | 9.0 |
| Cu                                    | 1.0  | —   |
| Fe                                    | 0.2  | 5   |
| Si                                    | 0.6  | —   |
| Li                                    | 1.0  | —   |
| Al                                    | Rest | —   |
| Tensile strength kg./cm. <sup>2</sup> | 57   | —   |
| Elongation %                          | 10   | 10  |

The alloy may also contain two or more of the auxiliary metals.

## Example 5

|                                       |      |      |      |    |
|---------------------------------------|------|------|------|----|
| Mg                                    | 2.5  | 2.5  | 2.5  | 15 |
| Zn                                    | 9.0  | 9.0  | 9.0  | —  |
| Cu                                    | 1.0  | 1.0  | 1.0  | —  |
| Fe                                    | 0.2  | 0.2  | 0.2  | —  |
| Si                                    | 0.6  | 0.6  | 0.6  | —  |
| Co                                    | 0.5  | 1.0  | 2.0  | —  |
| Mn                                    | 0.8  | 0.8  | 0.8  | —  |
| Al                                    | Rest | Rest | Rest | —  |
| Tensile strength kg./cm. <sup>2</sup> | 61.2 | 63.6 | 60.8 | —  |
| Elongation %                          | 16.6 | 11.6 | 10.0 | —  |

## Example 6

|                                       |      |      |      |    |
|---------------------------------------|------|------|------|----|
| Mg                                    | 2.5  | 2.5  | 2.5  | 25 |
| Zn                                    | 9.0  | 9.0  | 9.0  | —  |
| Cu                                    | 1.0  | 1.0  | 1.0  | —  |
| Fe                                    | 0.2  | 0.2  | 0.2  | —  |
| Si                                    | 0.6  | 0.6  | 0.6  | 30 |
| Mo                                    | 0.5  | 1.0  | 2.0  | —  |
| Mn                                    | 0.8  | 0.8  | 0.8  | —  |
| Al                                    | Rest | Rest | Rest | —  |
| Tensile strength kg./cm. <sup>2</sup> | 58.7 | 60.3 | 54.1 | —  |
| Elongation %                          | 20.0 | 12.0 | 12.6 | 35 |

## Example 7

|                                       |      |      |      |      |
|---------------------------------------|------|------|------|------|
| Mg                                    | 2.5  | 2.5  | 2.5  | 2.5  |
| Zn                                    | 9.0  | 9.0  | 9.0  | 9.0  |
| Cu                                    | 1.0  | 1.0  | 1.0  | 1.0  |
| Fe                                    | 0.2  | 0.2  | 0.2  | 0.2  |
| Si                                    | 0.6  | 0.6  | 0.6  | 0.6  |
| Li                                    | 0.1  | 0.2  | 0.4  | 0.6  |
| Mn                                    | 0.8  | 0.8  | 0.8  | 0.8  |
| Al                                    | Rest | Rest | Rest | Rest |
| Tensile strength kg./cm. <sup>2</sup> | 62.5 | 62.9 | 65.2 | 65.8 |
| Elongation %                          | 18.5 | 14.0 | 12.4 | 8.0  |

## Example 8

|                                       |     |   |   |      |
|---------------------------------------|-----|---|---|------|
| Mg                                    | 2.5 | — | — | —    |
| Zn                                    | 8.0 | — | — | —    |
| Cu                                    | —   | — | — | 1.0  |
| Fe                                    | —   | — | — | 0.3  |
| Si                                    | —   | — | — | 0.8  |
| Mo                                    | —   | — | — | 1.5  |
| Al                                    | —   | — | — | Rest |
| Tensile strength kg./cm. <sup>2</sup> | 56  | — | — | —    |
| Elongation %                          | 11  | — | — | 60   |

## Example 9

|                                         |      |
|-----------------------------------------|------|
| Mg                                      | 2.5  |
| Zn                                      | 9.0  |
| Cu                                      | 1.0  |
| 5 Fe                                    | 0.3  |
| Si                                      | 0.8  |
| Co                                      | 2.0  |
| Li                                      | 0.7  |
| Al                                      | Rest |
| 10 Tensile strength kg./cm <sup>2</sup> | 58   |
| Elongation %                            | 10   |

## Example 10

|                                      |      |
|--------------------------------------|------|
| 15 Mg                                | 3.0  |
| Zn                                   | 9.0  |
| Cu                                   | 0.8  |
| Fe                                   | 0.2  |
| Si                                   | 0.6  |
| 20 Mo                                | 2.5  |
| Li                                   | 1.0  |
| Al                                   | Rest |
| Tensile strength kg./cm <sup>2</sup> | 57   |
| Elongation %                         | 11   |

- 25 As to be seen from the above examples, the new alloy according to the invention has a very great tensile strength and a very great elongation which are hardly obtained in known aluminium alloys.

As to mutual actions of the elements for the new alloy, it is supposed as follows. A part of magnesium may combine with silicon to form magnesium silicide, and another part of magnesium may be alloyed with a part of zinc and a part of aluminum to form various three elemental alloys of different percentage. Further copper may be alloyed with iron. These chemical compound and alloys may crystal out in the main element, viz., aluminium and may be uniformly distributed therein. Further, when manganese is employed, this manganese and titanium not only act as reducing agents, but also hinders the growth of particles of zinc-manganese-aluminium alloys and also of copper-iron alloy so that the distribution of the alloys may be promoted.

Also it is deemed that the smaller percentage of iron gives a greater strength and elongation and this fact is supposed that iron may be detrimental to the natures, and this drawback is eliminated by using silicon or silicon and manganese in a greater percentage.

What I claim is:—

An aluminium alloy containing 2 to 5% magnesium, 6 to 14% zinc, .3 to 2% copper, .01 to 5% iron, .1 to 1% silicon, the silicon content being always greater than the iron content, .1 to 1% manganese and the rest aluminium.

YONOSUKE MATUENAGA.